

May 5, 1970

MAKOTO YOSHIDA ETAL

3,510,306

DEVELOPING PROCESS FOR COLOR PHOTOGRAPHY

Filed June 8, 1966



INVENTORS  
MAKOTO YOSHIDA  
BY MOMOTOSHI TSUDA

*Sughrue, Rothwell, Min, Zion & Macpeak*  
ATTORNEYS

1

3,510,306  
DEVELOPING PROCESS FOR COLOR  
PHOTOGRAPHY

Makoto Yoshida and Momotoshi Tsuda, Kanagawa,  
Japan, assignors to Fuji Shashin Film Kabushiki  
Kaisha, Kanagawa, Japan

Filed June 8, 1966, Ser. No. 556,238

Claims priority, application Japan, June 9, 1965,  
40/33,775

Int. Cl. G03c 7/36

U.S. CL. 96—55

6 Claims 10

### ABSTRACT OF THE DISCLOSURE

The invention is directed to an improved color photographic developing process in which a coupler of the formula



is reacted with the oxidation product of an aromatic primary developer. The couplers of this invention are yellow couplers capable of forming yellow dyes, having excellent spectral absorption characteristics for providing ideal yellow images and have good silver removing properties.

The present invention relates to color photography and more particularly to a color photographic developing process using a color developing solution containing an improved coupler.

The use of such a coupler as forms dye images by the reaction thereof with the oxidation product of an aromatic primary amine developer in a color photographic development is known and there are many patents concerned with such couplers. Such a coupler will be coupled with the oxidation product of an aromatic primary amine to form a dye which is insoluble in water or a usual developing solution, whereby dye images can be left in the photographic emulsion layer. Such a coupler may be added in a developing solution or may be incorporated in a photographic emulsion layer before exposure. The coupler in this invention is of the type which is added to a developing solution.

This type of coupling process is usually a subtractive color process, wherein the couplers capable of forming cyan, magenta and yellow dyes are used.

Couplers for color photography are required to form, by color development, dyes having desired spectral absorption characteristics.

Ideally speaking, in particular, a yellow coupler must absorb completely blue lights and transmit completely green and red lights. However, many of the conventionally used couplers are deficient in such characteristics. Further, in the case of processing a photographic emulsion layer containing a yellow coupler, it is, after a first development, exposed in blue light, subjected to a yellow color development, and then bleached and fixed to provide yellow images. But in this case it frequently happens that the reduced silver remains in the bleaching step caused by the slow oxidation of the reduced silver and the silver remains in the yellow image without being removed completely in the fixing step. Hereinafter, the phenomenon is called insufficient silver removal. This reduces extremely the transparency of the yellow image.

An object of this invention is to provide a color photographic developing process using an improved yellow coupler capable of forming a yellow dye having the ex-

2

cellent spectral absorption characteristics for providing ideal yellow images and having good silver-removing property.

According to the present invention, the color developing solution contains a yellow coupler represented by the general formula



wherein X represents a halogen atom, an alkyl group, a trifluoromethyl group, an alkoxy group, an acylamino group or an aryloxy group; Y represents a hydrogen atom or above-mentioned group X; and Z represents a hydrogen atom or a halogen atom.

The above alkyl group may be, for example, methyl, ethyl, and propyl groups. The above-mentioned alkoxy group may be, for example, methoxy, ethoxy and propoxy groups. The acylamino group may be, for example, acetamino, propionamino, benzoylamino, toluenecarboamino, methanesulfoamino, benzenesulfonamino, and toluenesulfonamino groups. The aryloxy group may be, for example, phenoxy and tolyloxy groups.

It has been known that benzoylacetanilide is useful as a yellow coupler but the dye image obtained by using the yellow coupler has a bad silver-removing property and reduced spectral absorption characteristics.

Furthermore, 2-methylbenzoylacetanilide is described in "J. of the American Chemical Society," vol. 79, page 2920, but the silver-removing property of the coupler is bad and, as shown in the accompanying drawing, the spectral absorption characteristics of the thus obtained colored image are unsuitable.

The accompanying drawing contains a single figure which is a graphical plot of the absorption curves of a material of this invention and other materials.

In the drawing there are shown comparatively the spectral absorption curve A of a dye image formed by the oxidizing coupling of 2-methylbenzoylaceto-(2-chloro) anilide which is a typical coupler used in this invention and a color developer, 4-N,N-diethylaminoaniline; the spectral absorption curve B of the dye image obtained from a control coupler, benzolacetanilide and the above-mentioned color developer; and the spectral absorption curve C of the dye image obtained from another control coupler, 2-methylbenzoylacetanilide and the above-mentioned color developer. In the graph, the vertical axis is graduated for Optical Density and the horizontal for wavelength of light.

From the curves it will be understood that the dye image obtained from the coupler of this invention has less undesirable components which absorb in the green range and has very excellent absorption characteristics.

Moreover, it will be also understood that the coupler of this invention has very preferable property in silver removal as shown below.

That is, the silver-removing property is shown numerically by the ratio of the silver density, measured by using a red filter, to the sum of the densities of the dye image and silver image, measured by using a blue filter, as follows

$$\frac{\text{red light density (D}_R\text{)}}{\text{blue light density (D}_B\text{)}} = \text{numerical value}$$

The numerical values are compared for the above-mentioned dye images (A), (B), and (C) corresponding to the spectral absorption curves shown in the accompanying drawing, and also for the dye image (D), formed by the oxidizing coupling of 4-methylbenzoylaceto-(2-fluoro)anilide, which is also one of the couplers used in

this invention and 4-N,N-diethylaminoaniline; the dye image (E) obtained from 2-methylbenzoylaceto-(4-(4-toluenesulfonamido)anilide and the above-mentioned developer; and the dye image (F) obtained from 3-methylbenzoylaceto-(2-methoxy)anilide and the above-mentioned developer. The results are as follows:

| Dye image | DB   |      |      |      |
|-----------|------|------|------|------|
|           | 0.5  | 1.0  | 1.5  | 2.0  |
| A         | 0.21 | 0.17 | 0.16 | 0.14 |
| B         | 0.35 | 0.28 | 0.16 | 0.25 |
| C         | 0.36 | 0.30 | 0.28 | 0.26 |
| D         | 0.22 | 0.19 | 0.17 | 0.16 |
| E         | 0.22 | 0.19 | 0.17 | 0.25 |
| F         | 0.23 | 0.20 | 0.18 | 0.16 |

From the results it will be clear that the couplers used in this invention give very good silver removing property. The good silver-removing property shows up in the ex-

cellent transparency of the thus obtained dye image, which is very profitable for color reproduction.

The reason that the dye images obtained from the couplers of this invention have the spectral absorption characteristics and very good silver-removing property may be considered to be based on the chemical structure thereof in that the benzoyl nucleus has a methyl group and the anilide nucleus has as substituents at least one of the group consisting of halogen atoms, alkyl groups, trifluoromethyl groups, alkoxy groups, acylamino groups or aryl oxy groups.

In particular, as is clear from the examples below, the coupler having a methyl group at the 2-position of the benzoyl nucleus and one of the above-mentioned substituents at the 2-position of the anilide nucleus is excellent.

The use of the couplers shall not be limited to natural color photography but they may be used for obtaining mono-color images or two-color images.

Examples of the yellow couplers useful in this invention are as follows:

| Formula No. | Coupler formula | Melting point, °C. |
|-------------|-----------------|--------------------|
| 1           |                 | 94-95              |
| 2           |                 | 65                 |
| 3           |                 | 125                |
| 4           |                 | 82                 |
| 5           |                 | 156                |
| 6           |                 | 154                |
| 7           |                 | 121-122            |
| 8           |                 | 57-58              |
| 9           |                 | 141                |
| 10          |                 | 141                |
| 11          |                 | 92                 |
| 12          |                 | 109                |

| Formula No. | Coupler formula | Melting point, °C. |
|-------------|-----------------|--------------------|
| 13          |                 | 147                |
| 14          |                 | 145                |
| 15          |                 | 73-74              |
| 16          |                 | 92                 |
| 17          |                 | 142                |
| 18          |                 | 158                |
| 19          |                 | 118                |
| 20          |                 | 82                 |
| 21          |                 | 121                |
| 22          |                 | 98                 |
| 23          |                 | 164                |
| 24          |                 | 129                |
| 25          |                 | 132                |

The above couplers may be prepared, for example, as follows:

#### PREPARATION 1

2-methylbenzoylacetophenone-(2-chloro) anilide—(Formula 1)

Into a 1 liter three-necked flask equipped with a stirrer, a thermometer and an outlet for ethanol were charged 1 mole of ethyl-2-methylbenzoylacetate, 1 mole of o-chloroaniline and 250 ml. of xylene. The system was heated to 140-150° C. in an oil bath with stirring to distill off by-product ethanol. After about 3 hours, 80% of ethanol was distilled off. The reaction was then stopped and the product was cooled, poured in 300 ml. of petroleum ether, and allowed to stand for one night in a cold place to precipitate a white crystalline product which was filtered by suction, washed with 1000 ml. of petroleum ether and

then recrystallized using 2000 ml. of ligroin. The yield was 82% and the melting point of the crystal was 94-95° C.

#### PREPARATION 2

2-methylbenzoylacetophenone-(2-fluoro) anilide—(Formula 4)

65 The same procedure as in Preparation 1 was repeated using o-fluoroaniline instead of o-chloroaniline to provide a white crystalline product which was recrystallized by using methanol. The yield for the product was 55% and the melting point thereof was 82° C.

#### PREPARATION 3

4-methylbenzoylacetophenone-(2-fluoro) anilide—(Formula 12)

The procedure as in Preparation 1 was repeated using 75 1 mole of ethyl-4-methylbenzoylacetate, 1 mole of o-

fluoroaniline, and 300 ml. of xylene to provide a white crystalline product which was recrystallized by using methanol. The yield was 49% and the melting point of the crystal was 109° C.

## PREPARATION 4

2-methylbenzoylaceto-(2-ethoxy)anilide—(Formula 16)

The same procedure as in Preparation 1 was repeated using o-ethoxyaniline instead of o-chloroaniline to give a white crystalline product which was recrystallized by using acetonitrile. The yield of the product was 48% and the melting point thereof was 92° C.

## PREPARATION 5

2-methylbenzoylaceto-(4-(4-toluenesulfonamide) anilide—Formula 17)

The same procedure as in Preparation 1 was repeated using 4-(toluenesulfonamido)aniline instead of o-chloroaniline to provide a white crystalline product which was recrystallized by using methanol. The yield of the product was 53% and the melting point thereof was 142° C.

## PREPARATION 6

3-methylbenzoylaceto-(2-methoxy)anilide—(Formula 20)

The same procedure as in Preparation 1 was repeated using 1 mol of ethyl-3-methyl-benzoyl acetate, 1 mol of o-anisidine and 300 ml. of xylene to provide a white crystal, which was recrystallized by using a mixed solvent of ligroin and ethanol (1:1). The yield for the product was 75% and the melting point thereof was 82° C.

The invention will further be described with reference to the following examples.

## EXAMPLE 1

A gelatino silver bromo-iodide emulsion which had not been color sensitized was applied to a cellulose acetate film to provide a test sample having a blue sensitive emulsion layer. The material was subjected to differential exposures by means of an NSG type actinometer. Then, using a yellow color developing solution having the following composition:

Sodiumsulfite—5.0 g.

4-N,N-diethylaminoaniline sulfite—3.0 g.

Potassium bromide—1.0 g.

Potassium iodide (aq. 0.1% soln.)—5.0 ml.

Glauber's salt—20 g.

2-methylbenzoylaceto-(2-chloro)-anilide (Formula 1)—1.0 g.

Sodium hydroxide—2.5 g.

Water to make up—1000 ml.

the material was subjected to the following color development as usual:

First development 24° C.—5 min.

Water washing—2 min.

Reversal blue exposure—200 GMC.

Yellow color development—5 min.

Water washing—2 min.

Bleaching—2 min.

Water washing—2 min.

Fixing—2 min.

Water washing—2 min.

By this procedure, a positive image of yellow dye having very good transparency was obtained. The spectral absorption curve of the dye image is shown in the accompanying drawing as Curve A.

## EXAMPLE 2

The same test sample as in Example 1 was subjected to the same differential exposure as in the example and then color developed as in the example using 2-methylbenzoylaceto-(2-ethoxy)anilide (Formula 16) instead of

3-methylbenzoylaceto-(2-chloro)anilide (Formula 1) to provide a positive image of the yellow dye having an absorption maximum of 438 nm. and very good transparency.

## EXAMPLE 3

The same test sample as in Example 1 was subjected to differential exposure and, using a yellow color developing solution having the following composition, was color developed as in Example 1:

## Developing solution

Glauber's salt—80 g.

Potassium bromide—1 g.

Sodium sulfite—5 g.

Potassium iodide (0.1% soln.)—16 ml.

Sodium hydroxide (10% soln.)—28 ml.

Hexylene glycol—20 ml.

2-methylbenzoylaceto-(2-fluoro)anilide (Formula 4)—1.5 g.

4-N,N-diethylaminoaniline sulfite—3 g.

1-phenyl-3-pyrazolidone—0.1 g.

By the procedure, a positive image of yellow dye having an absorption maximum of 445 nm. and very good transparency was produced.

## EXAMPLE 4

The same procedure as in Example 1 was repeated using as the coupler 4 - methylbenzoylaceto-(2-fluoro) anilide (Formula 12) instead of 2-methylbenzoylaceto-(2-chloro)anilide to give a positive image of yellow dye having an absorption maximum of 448 nm. and very good transparency.

## EXAMPLE 5

The same procedure as in Example 1 was repeated using as the coupler 2-methylbenzoylaceto(4-(4-toluenesulfonamido)anilide (Formula 17) instead of 2-methylbenzoylaceto-(2-chloro)anilide to provide a positive image of yellow dye having an absorption maximum of 442 nm. and very good transparency.

What we claim is:

1. In a color photographic developing process wherein a developer solution containing a coupler and an aromatic primary amine developer is applied to a silver halide photographic emulsion, forming dye images by the reaction of the coupler with the oxidation product of the aromatic primary amine developer, the improvement comprising color developing by application of a solution containing a coupler represented by the general formula:



wherein X represents a member selected from the group consisting of a halogen atom, an alkyl group, a trifluoromethyl group, an alkoxy group, an acylamino group and an aryloxy group; Y represents a member selected from the group consisting of a hydrogen atom, a halogen atom, an alkyl group, a trifluoromethyl group, an alkoxy group, an acylamino group and an aryloxy group and Z represents a member selected from the group consisting of a hydrogen atom and a halogen atom.

2. The color photographic developing process as claimed in claim 1 wherein said alkyl group is selected from the group consisting of methyl, ethyl and propyl.

3. The color photographic developing process as claimed in claim 1 wherein said alkoxy group is selected from the group consisting of methoxy, ethoxy and propoxy.

4. The color photographic developing process as claimed in claim 1 wherein said acylamino group is selected from the group consisting of acetamino, propionamino, benzo-

ylamino, toluenecarboamino, methane-sulfoneamino, benzenesulfoneamino and toluenesulfonamino.

5. The color photographic developing process as claimed in claim 1 wherein said aryloxy group is selected from the group consisting of phenoxy, tolyloxy.

6. The color photographic developing process as claimed in claim 1 wherein said coupler has a methyl group at the 2-position of the benzoyl nucleus and is substituted by one of the members X, Y and Z at the 2-position of the anilide nucleus.

## References Cited

## UNITED STATES PATENTS

2,513,190 6/1950 McQueen ----- 96—100

## FOREIGN PATENTS

5 595,314 12/1947 Great Britain.

J. TRAVIS BROWN, Primary Examiner